

Oct. 5, 1965

D. E. READ ET AL

3,210,240

SIZING PAPER WITH A FOAMED STARCH

Filed July 16, 1963



INVENTORS:  
DOUGLAS E. READ  
WILLIAM B. CRANFORD  
ANTHONY J. PETRICOLA

BY

*D. E. Read*

ATTORNEY

3,210,240

## SIZING PAPER WITH A FOAMED STARCH

Douglas E. Read, William B. Cranford, and Anthony J. Petricola, Hawkesbury, Ontario, Canada, assignors to Canadian International Paper Company, Montreal, Quebec, Canada, a corporation of Canada  
Filed July 16, 1963, Ser. No. 295,386  
6 Claims. (Cl. 162—175)

This invention relates to the manufacture of paper having improved surface qualities. More particularly, it relates to a process for improving newsprint, newsrot, novel news, directory, catalog and similar papers.

Many press rooms using newsprint or the like are converting to offset presses. In such presses, the ink, which is considerably more viscous and adhesive than the ink generally used in letterpress printing, is transferred to the paper from a rubber blanket. An appreciable force is required to remove the printed paper from the rubber blanket, because of the nature of the ink, and such force and the ink cooperate to pick up on the blanket any relatively loose fibers occurring on the surface of the paper and to accumulate such pick-up or lint on the blanket and the printing plate. This ultimately causes a deterioration of the printing quality and eventually forces a shutdown of the press for clean-up. This problem is usually satisfactorily mitigated when the paper is newsprint by doing the offset printing on the wire side of the sheet from which loose fibers are relatively absent, but it is not always possible or convenient to print the wire side of the sheet only and the problem is a significant one with respect to the top-side or felt-side of the sheet.

Accordingly, there is a need to develop means capable of bonding top surface fibers relatively firmly to the main body of a sheet of paper useful in offset printing. These means must be cheap or the economic advantage of using a paper such as newsprint will be lost. In addition, certain deleterious side effects must be avoided. Thus, for instance, since many newsprint offset inks "dry" mainly by absorption, the porosity of the sheet must be reasonably maintained. Again, since Customs' regulations restrict the water penetration resistance of papers which they permit to be imported into the U.S. duty-free, they practically eliminate the use of rosin size or water resistant film coatings on such papers.

It is, therefore, an object of the present invention to enable the manufacture of the newsprint and other comparable paper stocks having an improved bonding between the top surface fibers and the bodies of such papers simply and inexpensively and with substantially no change in their characteristics of porosity and water penetration resistance.

It has heretofore been proposed to apply an uncooked starch to the top surface of a travelling paper web before it is heat dried. See co-pending U.S. Serial No. 178,874, filed March 12, 1962, and now abandoned in favor of continuation-in-part application Serial No. 331,643, filed December 11, 1963. The starch, in the form of an aqueous slurry with or without an admixture of papermaker's alum, is not highly viscous and, therefore, does not interfere appreciably with the removal of water from the sheet on, for instance, the wire of a Fourdrinier paper machine. Furthermore, the uncooked starch particles tend to remain near the top surface of the sheet where they are needed, when, upon entering the dryer section of the machine, the combination of heat and moisture causes the particles to swell, become sticky, and to form fiber-starch-fiber linkages which bond the loose surface fibers to the main body of the sheet.

A further refinement is now proposed, one which greatly minimizes the rather large addition of water to the paper sheet which is inherent in the use of a starch slurry

the vehicle of which is water and one which, thereby, affords not only greater economy in paper production, but also provides for a more even and better surface sizing of the paper as established by iodine developing. Moreover, such refinement permits the use of minimal quantities of cooked or uncooked starches or mixtures thereof per ton of paper, i.e., about 10 to 20 lbs. of starch per air dried ton of a paper such as newsprint.

In accordance with the present invention, starches—whether raw, cooked, modified, or any mixture thereof—are foamed by means of compressed air and with the aid of wetting agents or surfactants; the starch foam is dried by draining and the dried starch foam is applied to the paper sheet (without any submersion or immersion thereof in the foam) by conventional means such as applicator rolls, scrapers, doctor blades, or any combinations thereof, or is metered onto them oving sheet just ahead of the nip of press rolls.

Thus, for example, two aqueous solutions were made up as follows:

- (1) 100 gm./l. dispersion of an uncooked modified (hydroxyethylated) starch commercially available as SLS 240  
(2) 9 gm./l. sodium lauryl sulfate (an anionic wetting agent)

These were metered to the bottom of a column 2 inches in diameter by 3 feet high. Compressed air was also admitted to the bottom of the column and the resulting foam was led from the top of the column to a small size press having a nip formed by an upper steel roll and a lower rubber roll. A 15" wide web of newsprint paper was pulled into, through, and out of the size press nip at about 100 ft./min. and, at the same time, the foam was applied to the top roll so as to form a bead of foam in the nip between the steel roll and the newsprint. The pumping rates of the two solutions entering the column were regulated so as to coat the web on its felt side with about 15 to 20 lbs. of the starch and about 1.8 lbs. of wetting agent per ton of newsprint. About 15 to 20% moisture was added to the newsprint in the process. The specific volume of the foam was about 20 times that of the liquid giving rise to the foam.

Again, in another example, two aqueous solutions were made up as follows:

- (1) 50 gm./l. dispersion of cooked corn starch cooled to about room temperature  
(2) 9 gm./l. sodium lauryl sulfate

These solutions were employed as were those in the first example. In this case, the rate of application of the starch was about 120 cc./min. and that of the wetting agent was about 60 cc./min. Subsequent testing showed the addition to the felt side of the web of about 21 lbs. of starch and the addition of about 24.4% more moisture to the web.

Further work has shown that, in some cases, it is preferable to add some carboxymethylcellulose to the starch to heighten viscosity slightly and to provide a trap in the line from the foaming column to the size press for assistance in drying the foam by draining excess liquid therefrom (the resulting foam is quite stable and is capable of standing in the open atmosphere for several hours with very little liquid drainage). In addition, it has shown that raw starch solutions of 10% or higher concentration can easily be foamed to volume/weight ratios of as high as 50/1 and that cooked starches of up to about 3.3% concentration can be foamed to volume/weight ratios of about 20/1, a reduction in concentration leading to an increase in ratio. Similarly, mixtures of up to about 3% cooked and about 7% raw starches

3 yield ratios favorably comparable to those attained with raw starch alone.

It is known that anionic surfactants are usually better foaming agents than either cationic or non-ionic surfactants, and sodium lauryl sulfate, commercially available as Sipon LSB or Sterling WA Paste, has been found to be by far the best of several tried, particularly when used in an amount equal to about 5% by weight of the starch.

For a still better understanding of the present invention, reference should be had to the attached sheet of drawing including FIGURES 1 and 2 and illustrating schematically two arrangements of equipment suitable for use in carrying out the process of the invention or, at least, the foam formation part of the process.

What is claimed is:

1. In the manufacture of a paper selected from the group consisting of newsprint, newsroto, novel news, directory, and catalog papers, a process of bonding two surface fibers of the paper to the body thereof comprising foaming starch dispersed in water by means of compressed air and with the aid of a wetting agent, draining the starch foam of excess water, and applying the drained starch foam to the paper at a rate equivalent to about 10 to 20 lbs. per ton of air dried paper.

- 2. The process of claim 1 wherein the starch is raw starch.
- 3. The process of claim 1 wherein the starch is cooked starch.
- 5. 4. The process of claim 1 wherein the starch is modified starch.
- 5. The process of claim 1 wherein the wetting agent is sodium lauryl sulfate.
- 6. The process of claim 5 wherein the wetting agent is about 5% by weight of the foamed starch.

10

References Cited by the Examiner

UNITED STATES PATENTS

|    |           |       |                   |       |         |
|----|-----------|-------|-------------------|-------|---------|
| 15 | 2,214,641 | 9/40  | Massey et al.     | ----- | 162—175 |
|    | 2,337,915 | 12/43 | Menger et al.     | ----- | 106—122 |
|    | 2,442,928 | 6/48  | MacMasters et al. | ----- | 106—122 |
|    | 2,666,718 | 1/54  | Davis             | ----- | 117—156 |
|    | 2,947,647 | 8/60  | Hart et al.       | ----- | 162—101 |

20 DONALL H. SYLVESTER, *Primary Examiner.*

MORRIS O. WOLK, *Examiner.*

UNITED STATES PATENT OFFICE  
CERTIFICATE OF CORRECTION

Patent No. 3,210,240

October 5, 1965

Douglas E. Read et al.

It is hereby certified that error appears in the above numbered patent requiring correction and that the said Letters Patent should read as corrected below.

Column 3, lines 18 and 19, for "bonding two surface" read  
-- bonding top surface --.

Signed and sealed this 23rd day of August 1966.

(SEAL)

Attest:

ERNEST W. SWIDER

Attesting Officer

EDWARD J. BRENNER

Commissioner of Patents